

June 4, 1968

J. VAN LAAR ET AL

3,387,161

## PHOTOCATHODE FOR ELECTRON TUBES

Filed Nov. 18, 1965

2 Sheets-Sheet 1



FIG.1



FIG. 2



FIG. 3

JOHANNES VAN LAAR  
JACOB J. SCHEER  
BY

BY  
Frank P. Jinfai  
AGENT

June 4, 1968

J. VAN LAAR ET AL

3,387,161

PHOTOCATHODE FOR ELECTRON TUBES

Filed Nov. 18, 1965

2 Sheets-Sheet 2



FIG. 5

INVENTORS  
JOHANNES VAN LAAR  
JACOB J.SCHEER  
BY  
*Frank R. Jaffari*  
AGENT

3,387,161

## PHOTOCATHODE FOR ELECTRON TUBES

Johannes van Laar and Jacob Jan Scheer, Emmasingel, Eindhoven, Netherlands, assignors to North American Philips Company, Inc., New York, N.Y., a corporation of Delaware

Filed Nov. 18, 1965, Ser. No. 508,499

Claims priority, application Netherlands, Dec. 2, 1964,  
64-13,961

9 Claims. (Cl. 313—94)

## ABSTRACT OF THE DISCLOSURE

An alkali metal activated photocathode comprising a heavily-doped p-type semiconductor of a III-V compound or mixed crystal thereof having an energy gap between 1.1 and 1.6 electron volts. A preferred embodiment comprises zinc-doped gallium-arsenide activated with cesium. Among the advantages are increased sensitivity in the red part of the spectrum.

This invention relates to a photocathode for an electron tube or device. In particular, it relates to a p-conductivity-type semiconductor photocathode or electron emitter activated with an alkali metal. An alkali metal is to be understood to mean herein also an alkali metal-oxygen combination constituting a substance of low work function.

The prior art photocathodes of the aforementioned composition have a comparatively high red sensitivity and their maximum quantum efficiencies may amount on an average to 20%. For a photocathode of the composition  $Cs_3Sb$ , for instance, the red boundary lies well over 6300 Å, and the maximum quantum efficiency of approximately 20% is attained after an abrupt rise of the sensitivity curve at approximately 4200 Å. For a photocathode of the composition  $Na_2KSb-Cs$ , the red boundary extends further out to approximately 8500 Å, but the sensitivity curve rises more slowly so that the maximum quantum efficiency of almost 40% is attained only at approximately 4200 Å. That wavelength at which the quantum efficiency amounts to 1% of the maximum efficiency of the sensitivity curve is assumed to be the red boundary. The red boundary consequently does not provide an absolute value for the sensitivity at that boundary. We have previously made some investigations on the photoelectric emission from p-type silicon, where we found that the red boundary of heavily-doped p-conducting silicon lies at approximately 5000 Å, but the maximum quantum efficiency was much too low for practical use. This is reported in Philips Research Reports, 17, 101-124 (1962).

The main object of our invention is to provide improved photocathodes which also have a favorable red boundary.

According to our invention, the photocathode comprises an alkali-metal-activated, heavily-doped, p-conductivity type III-V compound or mixed crystals of such compounds with an energy gap lying between 1.1 electron-volts (ev.) and 1.6 electron-volts (ev.). As usual, an III-V compound is understood to mean a practically equiatomic intermetallic compound of one of the elements (III) of the third column of the periodical system, viz., boron, aluminum, gallium, and indium, and one of the elements (V) of the fifth column of the periodical system, viz., nitrogen, phosphorus, arsenic, and antimony. In the case of mixed crystals, the quantity of III atoms present is substantially equal to that of the V atoms. According to a further feature of our invention, this AlIII-BV compound preferably consists of gallium arsenide having an acceptor concentration of at least  $1 \times 10^{18}$  per  $cm^3$  and preferably at least  $1 \times 10^{19}$  per  $cm^3$ . The maximum concentration amounts to approximately  $1 \times 10^{20}$ . A photocathode is thus obtained whose maximum quantum efficiency is at least equal to that of the known red-sensitive cathodes, and moreover the red boundary lies at a considerably greater wavelength than in the case of the known photocathodes. Still further, as a result of the abrupt rise of the sensitivity curve at the long-wave or red end, the overall sensitivity to white light is increased.

A preferred composition of our new photocathode is cesium-activated gallium arsenide containing  $4 \times 10^{19}$  zinc atoms per  $cm^3$ . The red boundary then lies upwards of 9200 Å, and the maximum quantum efficiency of approximately 40% is already attained at approximately 6000 Å. It is also possible to incorporate in the semiconductor other acceptor elements which produce p-conductivity in gallium arsenide in addition to the zinc. Examples of other acceptor elements are cadmium, mercury, or tellurium. A preferred mixed crystal of the invention comprises gallium arsenide with at the most a few percent, viz., 10%, of gallium phosphide or gallium antimonide.

The invention will now be described more fully with reference to the drawing, in which FIGS. 1 to 4 show different electron tubes containing a photocathode in accordance with the invention, and FIG. 5 illustrates spectral sensitivity curves comparing the sensitivities of various photocathodes.

As is well known in the art, there are various kinds of electron tubes or devices that employ photocathodes. These include photocells, photomultipliers, image intensifiers, iconoscopes, orthicons, and others. In most cases, the photocathode is mounted within an envelope, which is usually evacuated, in a position to receive the energizing photons of the incident light or radiation. The electron emissive part of the photocathode generally borders the evacuated space and emits electrons into it, which are collected by an anode or collecting electrode positioned a small distance away. The cathode and anode are connected across a source of potential and load in an external circuit. Where the photocathode is a crystal, the emissive surface may be a surface formed by cleaving the monocrystal along a crystal plane in a high vacuum or in air. Or the emissive surface may be formed by evaporating the material to form a thin layer on a conductive support. The alkali-metal activation, usually cesium, which has the lowest work function, is done in the conventional manner. A source of cesium is provided and cesium evaporated within the tube so as to form a deposit on the emissive surface of the cathode. Generally sufficient cesium is deposited until the photocathode exhibits a maximum sensitivity, which is usually achieved with an approximately monoatomic layer of the cesium.

FIG. 1 illustrates a tube of the type described in our previously-mentioned paper for making a crystal photocathode. It comprises a movable metal bellows 2 secured in a vacuum-tight manner to a quartz bulb 1. This metal part 2 supports a steel knife 3 by means of which part of a gallium arsenide monocrystal 4 is severed to expose a pure gallium arsenide surface. From a source (not shown), which may be of the type described in our previously-mentioned paper, an approximately monoatomic cesium layer 5 is applied to this freshly-cleaved surface by vaporization. A plate 6 serves as an anode. Upon exposure to radiation through the bulb 1, electrons are emitted from the cathode 4, 5.

FIG. 2 shows a modified phototube containing a curved molybdenum plate 8 arranged in an envelope. Onto the plate 8 is applied by vaporization a layer 9 of gallium

arsenide containing  $\frac{1}{2}\%$  of gallium phosphide. This may be done as follows. A fine granulated mixture of doped gallium arsenide and gallium phosphide is fed, in a good vacuum, into a heated tantalum crucible such that it immediately evaporates. This technique is known in the art as flush evaporation. The molybdenum substrate 8 is held at a temperature of about  $500^{\circ}\text{C}$ . to obtain the desired crystal structure. Afterwards, an approximately mono-atomic cesium layer is applied to the gallium arsenide layer 9 to produce the finished cathode. The anode is denoted by 10.

FIG. 3 shows a photomultiplier tube comprising a glass envelope 11 on one end of which is deposited by vaporization a cesium-activated gallium arsenide layer 12 having a thickness of 1000 Å. In the conventional way, the tube is also provided with a plurality of multiplier or dynode electrodes 13 and an anode 14 which constitute the remainder of the electrode system.

FIG. 4 illustrates an iconoscope with a gallium arsenide layer 16 deposited by vaporization on the flat end 15 of the envelope and serving as the light sensitive cathode. Of the remaining electrodes, only the thermionic cathode 17 is shown.

FIG. 5 compares the spectral sensitivity of the photocathode of the invention with several prior art cathodes. In the graph, the quantum efficiencies are plotted along the ordinate as a function of the wavelength of the exciting light in Å. The curve I was obtained with a monocrystal of cesium-activated gallium arsenide containing  $4 \times 10^{19}$  atoms of zinc/cm.<sup>3</sup> cleaved in a vacuum of  $10^{-10}$  torr. The curve II is typical of a  $\text{Na}_2\text{KSb}-\text{Cs}$  cathode, and the curve III is typical of a cathode  $\text{Cs}_2\text{Sb}$ . It is clearly apparent that the gallium arsenide photocathode of the invention has a particularly favorable quantum efficiency, a very long-wave red boundary and a steeply ascending sensitivity curve. The light outputs for white light for the photocathodes associated with the curves I, II and III are approximately 450  $\mu\text{a.}/\text{lumen}$ , 150  $\mu\text{a.}/\text{lumen}$  and 50  $\mu\text{a.}/\text{lumen}$ , respectively.

While we have described our invention in connection with specific embodiments and applications, other modifications thereof will be readily apparent to those skilled in this art without departing from the spirit and scope of the invention as defined in the appended claims.

What is claimed is:

1. A photocathode of an electron tube having an emissive surface portion, said portion comprising a p-type semiconductive material having an acceptor concentration of at least  $1 \times 10^{18}$  atoms/cm.<sup>3</sup> and selected from the group consisting of a III-V compound and mixed crystals of III-V compounds and having an energy gap between 1.1 and 1.6 electron volts and activated with an alkali metal, where III is an element selected from the group consisting of boron, aluminum, gallium, and indium, and V is an element selected from the group consisting of nitrogen, phosphorus, arsenic, and antimony.
2. A photocathode for an electron tube having an emissive surface portion, said portion comprising cesium-activated, p-type gallium arsenide having an acceptor concentration of at least  $1 \times 10^{18}$  atoms/cm.<sup>3</sup>
3. A photocathode as set forth in claim 2 wherein the acceptor concentration is at least  $1 \times 10^{19}$  atoms/cm.<sup>3</sup>.
4. A photocathode as set forth in claim 3 wherein the acceptor is selected from the group consisting of zinc, cadmium, tellurium and mercury.
5. A photocathode as set forth in claim 3 wherein the gallium arsenide is doped with approximately  $4 \times 10^{19}$  atoms of zinc/cm.<sup>3</sup>.
6. A photocathode as set forth in claim 1 wherein the material is gallium arsenide with no more than 10 percent of gallium phosphide or gallium antimonide.
7. A photocathode as set forth in claim 1 wherein the photoemissive portion is a cleaved surface of a monocrystal.
8. A photocathode as set forth in claim 1 wherein the photoemissive portion is a vapor deposited layer.
9. An electron tube containing a photocathode as defined in claim 1.

#### References Cited

##### UNITED STATES PATENTS

- |           |         |          |       |         |
|-----------|---------|----------|-------|---------|
| 3,098,168 | 7/1963  | Aigrain  | ----- | 313—346 |
| 3,114,070 | 12/1963 | Stratton | ----- | 313—346 |

##### OTHER REFERENCES

Philips Research Reports, vol. 17, pp. 101—124, 1962.

JAMES D. KALLAM, Primary Examiner.